

## UNITED STATES PATENT OFFICE

2,015,132

## VULCANIZED FIBER

James H. Young, Arden, Del., assignor to E. I.  
du Pont de Nemours & Company, Wilmington,  
Del., a corporation of Delaware

No Drawing. Application November 13, 1934,  
Serial No. 752,888

5 Claims. (Cl. 92—13)

This invention relates to vulcanized fiber, and more particularly to the manufacture of vulcanized fiber from chemical wood pulp.

In the manufacture of vulcanized fiber it has been the practice to treat with zinc chloride or other gelatinizing agents, paper made from bleached rag pulp of a high alpha cellulose content and a low viscosity in cuprammonium hydroxide. The dry sheets of paper are passed through a bath of zinc chloride or a mixture of zinc chloride with other chemicals to cause partial gelatinization of the cellulose fibers. The sheets are laminated to give the desired thickness, cured for a short time in air at room temperature, and then subjected to pressure and heat to insure good adhesion of the individual plies. The zinc chloride is gradually removed from the sheet by a system of counter-current washing. The final steps of the process are drying and pressing or rolling. A less dense product is made by using a rag pulp which will react slowly with the zinc chloride or by using sulfite wood pulp of high alpha cellulose content and low viscosity. In all instances it is essential for the success of this prior art method that the pulp used be one of low viscosity and high alpha cellulose content.

Attempts have also been made to use the various chemical wood pulps as a base material for vulcanized fiber. These wood pulps have been prepared by special cooking methods and have been given special treatments in order to produce a pulp corresponding in chemical properties to that of a satisfactory rag pulp, namely, a pulp of low viscosity and of high alpha cellulose content. The cost of preparing vulcanized fiber using these high alpha cellulose wood pulps is, however, much greater than it is for processes utilizing standard grades of wood pulp of low alpha cellulose content.

40 This invention has as an object a process for utilizing the inexpensive low alpha cellulose chemical wood pulps in the manufacture of vulcanized fiber. A further object is an improved process for making vulcanized fiber. Other objects will appear hereinafter.

45 These objects are accomplished by treating a chemical wood pulp of low alpha cellulose content but of high viscosity with mercerizing caustic, cutting the fibers to reduce their length, forming the fibers into sheets of paper, and vulcanizing the fibers with zinc chloride as will be more fully described hereinafter.

50 The caustic treatment to which the pulp in my process is initially subjected, is the superficial mercerization of the fibers with strong caustic

as described in U. S. Patent 1,857,100. The pulp produced in accordance with this patent has, however, not found heretofore wholly successful use as a base material for vulcanized fiber because of the lack of knowledge of certain essential requirements and of procedural steps which are disclosed herein. Thus, I have found that the mentioned caustic treatment is effective in the present process only if this treatment is applied to pulps which are specially selected because of 10 their high viscosity. I have also discovered that it is essential to cut the fibers of the mercerized pulp to reduce the fiber length before forming the pulp into paper prior to the zinc chloride treatment. 15

The pulp which receives the above-mentioned mercerizing treatment should have a viscosity in cuprammonium hydroxide of from 700 to about 1200 centipoises. I prefer to use pulps having an alpha cellulose content below 88%. Such pulps 20 are known as low alpha cellulose pulps, since pulps containing more than 93% alpha cellulose are referred to in the art as high alpha cellulose pulps. The alpha cellulose content rises somewhat after the caustic treatment but is still usually outside the range for high alpha cellulose pulp. The initial viscosity of the pulp I use changes but slightly and, hence, is distinguished sharply from the high alpha cellulose pulps of 90 to 200 centipoises viscosity in cuprammonium. 30 For the purposes of the present invention, wood pulps which before the mercerizing treatment have a viscosity in cuprammonium below 700 centipoises are unsatisfactory because the vulcanized fiber made therefrom is quite brittle. 35

In addition to the requirements for viscosity mentioned above it is important that a bleached pulp be used in the first step of my process which consists in the mercerizing treatment described above. I have found that a mercerized bleached 40 chemical wood pulp of low alpha cellulose content and a high viscosity reacts with zinc chloride solutions in the same manner as a pulp prepared from cotton rags of a high alpha cellulose content and a low viscosity. The vulcanized fiber prepared 45 from my low alpha-high viscosity base has the same physical properties as vulcanized fiber prepared from the standard high alpha-low viscosity base made from cotton rag. Examples of suitable pulps are bleached sulfite, bleached sulfate 50 and bleached soda pulp. The best results are obtained with a bleached sulfite pulp.

The use of a bleached pulp is important not because of color but because of certain properties imparted by the bleaching process to the pulp. 55

The bleaching reduces the viscosity of the cellulose and also removes lignin which prevents the zinc chloride from having the required gelatinizing action on the cellulose.

5 The cutting of the fibers after the mercerizing treatment is an essential step in the present process. It is important to observe, however, that this step of cutting the fibers into short, blunt sections must be sharply distinguished from the 10 conventional beating of the fibers with a large amount of water. In the latter instance although the fiber length is modified by the hydration and by the fraying of the fiber ends through continual rubbing action, and although the freeness is considerably decreased the properties of the paper 15 or felt made from the fibers is radically different from those of the felted cut fibers of the present invention. The sheet prepared from the beaten fibers is quite dense. The hydrated fibers are 20 tightly cemented together and liquids are therefore absorbed but slowly. The sheet made from the cut crinkled fibers, on the other hand, will be weaker, of lower density and more absorbent. This sheet is much more absorbent than a sheet 25 made from unmercerized fibers cut to the same freeness as the crinkled mercerized fibers used in the present invention.

The value of the step of cutting the fibers used in my process will be apparent from the resulting 30 advantages mentioned below as compared to the disadvantages of using the uncut and unmercerized fibers. Cut unmercerized fibers could not of course be used at all because the sheet does not absorb enough zinc chloride to cause gelatinization. When the cut mercerized fibers are used there is markedly less shrinkage after removal of the zinc chloride and drying than when the sheet is made of long fibers. The directional shrinkage also is greatly reduced because of the more 35 heterogeneous deposition of the short cut fibers in the sheet. On the other hand, in the case of a sheet made from the long uncut fibers there is considerable directional shrinkage due to the alignment of the greater part of the fibers in the 40 machine direction. Furthermore, cutting increases the area of the cellulose fibers that can be attacked by the zinc chloride solution and 45 gelatinization is therefore more uniform.

The details for the superficial mercerization of 50 the fibers of the pulp is fully set forth in the patent referred to above. The ordinary low alpha cellulose chemical wood pulp of  $\frac{3}{4}$  to 4 mm. fiber length, which for the present purpose must have the high viscosity described above, is mixed 55 by efficient dispersing apparatus at high pulp consistencies, namely, consistencies from 15 to 20%, with sodium hydroxide of mercerizing activity. For the present purpose sodium hydroxide solutions of 10 to 18% concentrations at 60 room temperature are suitable.

The short time of the caustic treatment together with the small proportion of liquor to pulp prevents any drastic action of the caustic on the pulp and results in a superficially mercerized 65 crinkled pulp of high freeness. This mercerizing treatment of the high viscosity-low alpha cellulose pulp is essential in the present process. First, the surface of the fibers is changed so that the zinc chloride solution does not react so quickly 70 with the cellulose. Second, the curled condition of the pulp makes it possible to reduce materially the length of the fibers by cutting without substantially affecting the absorbency of the sheet prepared from the pulp. This is very important 75 because the shrinkage that occurs when the sheet

of fibers is treated with zinc chloride is very greatly reduced when the length of the fibers is shortened by cutting. If the pulp is not first mercerized and if it reacts with zinc chloride, it shrinks abnormally. Cutting the fibers of such 5 pulp lowers the absorbency of the sheet to such an extent that it does not impregnate thoroughly with the zinc chloride solution.

After the pulp has been freed from the mercerizing liquor, it is subjected to a cutting treatment in Hollander-type beaters or Jordans to reduce the fiber length. The fibers may be dyed at this stage if so desired. They may then be cut by a final Jordan treatment to reduce their length sufficiently to give good sheet formation with 15 standard paper making equipment and to prevent excessive shrinkage when the sheet is subjected to the gelatinization treatment with zinc chloride solution. The mechanical treatment of the pulp should be such that the freeness is reduced from 20 about 25 to 55 seconds to about 160 to 250 seconds. The method of measuring freeness is described in the patent of reference.

The paper web, made by standard methods from the pulp treated as described above, is then 25 passed through a solution of 70.5% zinc chloride at 50° C. The treated sheet may be rolled onto a mandrel to form tube stock or it may be used in a continuous process to produce thin sheets. Several sheets of paper may be treated simultaneously in the same bath and laminated into sheets by the application of pressure and heat, and the resulting multiple sheet is then washed and dried in a continuous operation. The treated tubes or sheets are washed in successively weaker solutions 30 of zinc chloride. The final traces of zinc chloride are removed by washing the material in running water. The length of time required for curing the fiber depends on the thickness of the sheet. The washed fiber is finally dried and pressed. 35

The following examples illustrate more specifically the method for practicing my invention:

#### Example I

A bleached sulfite chemical wood pulp of the 45 following measurable properties:

Viscosity in cuprammonium 790.8 centipoises  
Alpha cellulose content 86.17%  
Freeness 95 seconds

was treated with an 18% caustic soda solution as 50 follows:

Pulp 20 parts  
18% NaOH solution 80 parts  
Temperature of NaOH solution 25° C. 55

The time of treatment is preferably not greatly in excess of that necessary to wet thoroughly all of the fibers with the caustic solution. With suitable equipment this is usually accomplished in less than a minute and even within the range 60 of 15 to 30 seconds. When wet pulp is used instead of the dry pulp in the present example, it is necessary as more fully pointed out in the mentioned patent that the caustic concentration be adjusted to compensate for the known amount 65 of moisture in the pulp.

The pulp was intimately mixed with the caustic soda solution to produce a superficial gelatinization of each fiber and to loosen them from the sheet form. After being treated the pulp was 70 promptly washed free of caustic soda with water. The washed pulp was "puffed" due to the curling and crinkling of the fibers and on examination under the microscope it was noted that the individual fibers of the washed pulp had a crinkled 75

appearance and a circular cross section, in contrast to the straight ribbon-like appearance of the untreated fibers. The properties of the treated pulp were as follows:

5 Viscosity in cuprammonium 858.0 centipoises  
 Alpha cellulose content 90.50%  
 Freeness 31 seconds

10 The fiber length of the pulp was reduced by cutting in a Hollander-type beater until the freeness was 200 seconds. Sheets .0070" thick were made from this pulp and were dried at 100-110° C. The dry paper was immersed 10 seconds in a 70.5% zinc chloride solution at 50° C. The 15 treated sheets were rolled onto 3/4" diameter mandrels and cured for two hours in the air at room temperature. The tubes were then immersed in a 20% zinc chloride solution for 24 hours, removed from mandrels, and immersed in 20 a 10% zinc chloride solution for 72 hours. The tubes were then immersed in water for 72 hours and finally washed with running water for two hours at which point no precipitate formed when the tubes were immersed in a dilute solution of 25 ammonium hydroxide. The tubes were placed on a mandrel and dried at 65° C. They were then rolled and polished under standard conditions of pressure and speed. No fracture resulted during the rolling test, and no blisters or untreated spots 30 were evident. The physical properties of the finished vulcanized fiber follow:

Shrinkage 14.5%  
 Specific gravity 1.519  
 35 Hardness 44.2

#### Example II

A bleached sulfite chemical wood pulp of the following properties:

40 Viscosity in cuprammonium 1118.0 centipoises  
 Alpha cellulose content 85.7%  
 Freeness 80 seconds

45 was treated with an 18% solution of caustic soda using the procedure cited in Example I. The properties of the treated pulp were as follows:

Viscosity in cuprammonium 962.0 centipoises  
 Alpha cellulose content 93.2%  
 Freeness 47 seconds

50 The fiber length of the treated pulp was reduced by cutting in a Hollander type beater until the freeness was 163 seconds. Sheets were made and treated with zinc chloride as cited in Example I.

55 The finished vulcanized fiber tubes were very tough. The physical properties of the tubes were as follows:

Shrinkage 9.4%  
 Specific gravity 1.540  
 60 Hardness 49

#### Example III

A bleached sulfite chemical wood pulp of the following properties:

65 Viscosity in cuprammonium 790.8 centipoises  
 Alpha cellulose content 86.17%  
 Freeness 95 seconds

70 was treated with a 12% caustic soda solution as follows:

Pulp 20 parts

12% NaOH solution 80 parts { 9.6 parts NaOH  
                                                          70.4 parts H<sub>2</sub>O

75 The same procedure was used for treating the

pulp with caustic soda solution as was used for Example I. Properties of the treated pulp were as follows:

Viscosity in cuprammonium 914.0 centipoises  
 Alpha cellulose content 89.51%  
 Freeness 37 seconds

80 The fiber length of the pulp was reduced by cutting in a small Jordan engine until the freeness was 225 seconds. The same procedure was used for preparing the sheets and for the subsequent treatment with zinc chloride as was cited in Example I. The physical properties of the finished vulcanized fiber follow:

Shrinkage 12.0%  
 Specific gravity 1.538  
 Hardness 48

85 Any of the agents useful for fiber vulcanization may be used for my process. Other suitable gelatinizing agents are zinc chloride, calcium thiocyanate cold caustic soda, and metallic halides. Also, zinc chloride can be mixed with other metallic halides, hydrochloric acid, acetic acid, or sulfuric acid. I prefer, however, to use zinc 25 chloride alone.

90 It is important that the requirements in the above examples of viscosity and of reduction of fiber length after the mercerizing treatment be adhered to. For instance, in repeating the procedure of Example I, I reduced the fiber length so that the freeness was changed from 31 seconds to 60 seconds instead of to 200 seconds. The sheets had irregular distribution of the fibers (poor formation) and they were very absorbent. 35 They were treated with zinc chloride solution and made into tubes according to the procedure outlined in Example I.

95 The finished fiber contained blisters and the shrinkage resulting from the action of zinc chloride on the fibers was unusually great. The vulcanized fiber had the following characteristics, shrinkage 30.0%, specific gravity 1.500, and hardness 34.6.

100 The importance of the viscosity requirement is shown by the following: A bleached chemical wood pulp of 85.7% alpha cellulose content but with a viscosity of only 652.0 centipoises was given the caustic treatment described in Example I. The treated pulp had a viscosity in cuprammonium of 640.0 centipoises, an alpha cellulose content of 94.4% and a freeness of 22.6 seconds. The fiber length was reduced by cutting to a freeness of 200 seconds as before and the vulcanization with the zinc chloride was likewise conducted as in Example I. The tubes were fractured during rolling and polishing. Also the shrinkage resulting from the treatment with zinc chloride was 31.0%. Hardness and density tests could not be made because the tubes were too brittle to make satisfactory vulcanized fiber.

105 The method used for measuring the viscosity of cellulose in cuprammonium hydroxide solution is the Standard A. C. S., method described in the Analytical Edition of Industrial and Engineering Chemistry, vol. 1, Number 1, pages 49-51. Briefly, the determination consists of measuring the time in seconds required for a 1/8 inch diameter glass sphere to fall 15 centimeters through a 2.5% solution of cellulose in 70 cuprammonium hydroxide that contains 30 g. of copper, 165 g. of ammonia, and 10 g. of sucrose per liter (1000 cubic centimeters). The viscosity is generally expressed as centipoises which is calculated by means of a standard formula 75.

involving the factors of density of the glass sphere, density of the solution, time required for sphere to fall, and a known conversion constant. It is to be understood that the viscosity figures used in the claims refer to a viscosity determination made with cuprammonium in this manner.

Alpha cellulose is defined as that form of cellulose which is insoluble in an 18% caustic soda solution at 20° C. when the treatment of the pulp with the caustic soda is carried out by the standard procedure.

The hardness figures given in the examples are the results of tests given with a Rockwell hardness tester as follows: A 9.5 millimeter diameter steel ball under a load of 100 kilograms was pressed against the sample of vulcanized fiber for a period of 15 seconds at room temperature. The Rockwell hardness number recorded on the "B" scale of the instrument at the end of 15 seconds was the hardness value. A hard material shows a high reading and a soft material shows a low reading.

The details in my invention are subject to various modifications as will be understood by those skilled in the art. Instead of mercerizing bleached chemical wood pulps, unbleached chemical wood pulps may be mercerized as outlined above and subsequently bleached after most of the mercerizing liquor has been removed from the pulp. It is necessary that the viscosity in cuprammonium and alpha-cellulose content of the bleached pulp fall within the limits which I have established.

For preparing very tough vulcanized fiber that is not to be used for electrical insulation, I may blend unreactive fibers with the pulp prepared by my preferred process. The mercerized fibers will insure good absorbency in the sheet.

Any of the standard chemical pulping processes yielding a fully liberated wood pulp fiber may be used for preparing the pulp providing the specified viscosity in cuprammonium and alpha cellulose content are obtained, and the mercerized fibers are cut sufficiently to give a sheet that will not shrink unduly in the process.

My invention is useful for manufacturing a paper base for vulcanized fiber that is used in electrical insulating work. This base is characterized by uniformity, good absorbency, and the correct reactivity with zinc chloride solutions. These factors are of great importance in manufacturing any type of vulcanized fiber.

A particular advantage of this invention is that certain standard chemical wood pulps which are relatively cheap, as compared to rag pulp and high alpha cellulose wood pulps, can be made suitable for vulcanized fiber base by mercerizing the fibers. Chemical wood pulps have an advantage over rag pulp because their chemical properties can be regulated and controlled within narrow limits by the time, pressure and con-

centration of chemicals used during the cooking process. Also, a uniform source of wood is available, whereas rags represent a very heterogeneous collection that vary widely in chemical properties. My invention represents a further advantage to the manufacturer of vulcanized fiber in that he may purchase a pulp which is ready for conversion into paper. Another feature is that chemical wood pulps are not contaminated with solid metallic particles such as are found in cotton rags. These metallic particles are very detrimental to electrical insulation. Although elaborate systems of riffle boxes and screens are used to remove them, they are never completely removed so the final product has many weak spots. 15

As many apparently widely different embodiments of this invention may be made without departing from the spirit and scope thereof, it is to be understood that I do not limit myself to the specific embodiment thereof except as defined in the appended claims.

I claim:

1. A process for making vulcanized fiber which comprises treating chemical wood pulp having a viscosity of about 700 to about 1200 centipoises 25 with a mercerizing agent under conditions which produce a mercerized fiber having not less than 25 seconds and not more than 55 seconds freeness, cutting the fibers to reduce the freeness within the range of about 160 to about 250 seconds, forming the cut fibers into paper, and treating the paper with a gelatinizing agent.

2. A process for making vulcanized fiber which comprises treating bleached chemical wood pulps containing less than 88% alpha cellulose and having a viscosity of about 700 to about 1200 centipoises with sodium hydroxide of mercerizing activity to produce a pulp having a freeness of from about 25 seconds to 55 seconds, cutting the fibers to reduce the freeness within the range of about 160 seconds to about 250 seconds, forming the cut fibers into paper and treating the paper with a gelatinizing agent.

3. In a process for making vulcanized fiber, the steps which comprise reducing the fiber 45 length of crinkled mercerized wood pulp having a viscosity of about 700 to about 1200 centipoises, sufficiently to cause good sheet formation and prevent excessive shrinkage when the sheet is subjected to gelatinization treatment for vulcanization of the fiber, felting the cut fibers into a sheet, and treating the sheeted fibers with a gelatinizing agent.

4. A process for making vulcanized fiber which comprises cutting mercerized bleached wood pulp 53 of high viscosity and high freeness to a freeness substantially lower, felting the cut pulp into paper, and treating the paper with a gelatinizing agent.

5. Vulcanized fiber substantially identical with that obtained in accordance with the process set forth in claim 1.

JAMES H. YOUNG.